

Patented Nov. 3, 1931

1,830,465

# UNITED STATES PATENT OFFICE

ERNEST T. HANDLEY, OF AKRON, OHIO, ASSIGNOR TO THE FIRESTONE TIRE & RUBBER COMPANY, OF AKRON, OHIO, A CORPORATION OF OHIO

## METHOD PREVENTING WATER BAG DETERIORATION

No Drawing. Application filed March 31, 1930, Serial No. 440,634. Renewed May 26, 1931.

This invention relates to a method for preventing deterioration of water bags such as used in the curing of pneumatic tires.

In the manufacture of pneumatic tires or similar hollow rubber articles vulcanized in steam-heated molds, it is the practice to place an air or water bag made of rubber inside the tire during the cure to assist in forcing the rubber of the green or uncured tire, softened by the heat of vulcanization, properly into the mold cavity. Air bags, which are rubber bags filled with compressed air, have proven satisfactory for this purpose but in the last few years the bags have been filled with very hot water under pressure which not only forces the tire to properly fill the mold cavity, but also serves to cure the tire from the inside while the steam-heated mold cures the tire from the outside. This inside and outside heating or cure gives a more uniform and evenly vulcanized tire than was possible with the old air bag, however, the conditions to which the water bag is subjected tend to rapidly deteriorate it. This deterioration is primarily from the inside of the bag outwardly and is due to the oxidizing action of the free oxygen dissolved in the water circulated through the bag. The temperature and pressure of the circulating water assists this oxidizing action so that after several cures the bags become so rotten that they will not hold the necessary pressure of the circulating water.

It is an object of the invention to overcome the above difficulties of the prior art by the provision of an inexpensive efficient process which prevents the oxidation and deterioration of the water bags under the necessary conditions of temperature and pressure.

The above and other objects of the invention are achieved by the method herein described, it being understood that the invention is not limited to exact details thereof described.

It has been found that by adding sodium sulphite ( $Na_2SO_3$ ) to the circulating water the interior oxidation of the water bags is substantially prevented and that the life of the water bags is materially increased.

In practicing the invention one-half ounce

of sodium sulphite will sufficiently deoxidize one gallon of circulating water so that it may be circulated through the water bags at ordinary vulcanization temperature and pressure without deterioration of the bags.

The above figures are, or course, for general conditions and may be widely varied in actual practice as the temperature and pressure of the circulating water and the composition of the water bag is changed.

The sodium sulphite may be introduced into the circulating water in any desired manner, such as dissolving it in water to give a concentrated solution and continually or periodically injecting the concentrated water solution into the circulating water to give the determined concentration therein or by passing the circulating water through a bed or filter of the sodium sulphite crystals or by merely dumping the sodium sulphite crystals into the circulating water.

The treated circulating water can be continuously used for a plurality of cures without loss of the properties thereof. Any necessary loss in the amount of the circulating water can be periodically replenished. However, if necessary or desirable the treated circulating water may be used for one cure or for only a short time as the sodium sulphite is inexpensive.

While the invention has been particularly described with respect to the manufacture of pneumatic tires it is evident that the principles thereof may be applied to the manufacture of any curable bodies which are forced into the molds by a water bag. Again the principles of the invention may be applied wherever hot water under pressure comes in contact with rubber.

As many other changes could be made in the process, it is intended that all matter contained in the above description shall be interpreted as illustrative only and not in a limiting sense, accordingly various modifications and applications of the invention can be resorted to without departing from the spirit of the invention or the scope of the appended claims.

What is claimed is:

1. In the manufacture of pneumatic tires

that method which comprises placing a water bag inside the green tire casing, placing the casing and bag in a heated mold, providing water for circulation through said water bag, placing sodium sulphite in the water to deoxidize the same, and circulating said deoxidized water through said bag under heat and pressure.

2. In the manufacture of moldable articles that method which comprises placing a water bag inside the green moldable article, placing the moldable article and bag in a heated mold, providing water for circulation through said water bag, placing sodium sulphite in the water to deoxidize the same, and circulating said deoxidized water through said bag under heat and pressure.

3. In the manufacture of moldable articles that method which comprises placing a water bag adjacent the green moldable article, placing the moldable article and bag in a heated mold, providing water for circulation through said water bag, placing sodium sulphite in the water to deoxidize the same, and circulating said deoxidized water through said bag under heat and pressure.

4. In the manufacture of pneumatic tires that method which comprises placing a water bag inside the green tire casing, placing the casing and bag in a heated mold, providing water to fill said water bag, placing sodium sulphite in the water to deoxidize the same, and filling said bag with said deoxidized water under heat and pressure.

5. In the manufacture of moldable articles that method which comprises placing a water bag inside the green moldable article, placing the moldable article and bag in a heated mold, providing water to fill said water bag, placing sodium sulphite in the water to deoxidize the same, and filling said bag with said deoxidized water under heat and pressure.

6. In the manufacture of pneumatic tires using rubber water bags for curing, that method which comprises forming a solution of sodium sulphite, and circulating said solution under heat and pressure through the water bag used in the cure whereby the oxidation of the interior of the water bag is prevented.

7. In the manufacture of pneumatic tires using rubber water bags for curing, that method which comprises forming a solution of sodium sulphite, and circulating said solution through the water bag used in the cure whereby the oxidation of the interior of the water bag is prevented.

8. In the manufacture of pneumatic tires using rubber water bags for curing, that method which comprises forming a solution of sodium sulphite, heating said solution, and circulating said solution under pressure through the water bag used in the cure whereby the oxidation of the interior of the water bag is prevented.

9. In the vulcanization of rubber articles using water bags for curing, that method which comprises circulating a solution of sodium sulphite through the water bag.

10. In the vulcanization of rubber articles using water bags for curing, that method which comprises heating a solution of sodium sulphite and introducing said solution into said water bag.

11. In the vulcanization of rubber articles using water bags for curing, that method which comprises circulating a solution of a sulphite of an alkali metal through the water bag.

12. In the vulcanization of rubber articles using water bags for curing, that method which comprises heating a solution of a sulphite alkali metal, and introducing said solution into said water bag.

13. In the vulcanization of rubber articles using water bags for curing, that method which comprises circulating water and a deoxidizing agent through the water bag.

14. In the vulcanization of rubber articles using water bags for curing, that method which comprises heating water and a deoxidizing agent, and introducing same into said water bag.

15. In the vulcanization of rubber articles using water bags for curing, that method which comprises dissolving a soluble reducing agent in water, heating said solution, and introducing said solution into said water bag.

ERNEST T. HANDLEY.

100

105

110

115

120

125

130